# EUROPEAN PATENT SPECIFICATION

(11) **EP 2 733 228 B1**
(45) Date of publication and mention of the grant of the patent: **19.06.2019**
(21) Application number: 11869574.1
(22) Date of filing: 15.07.2011
(51) Int. Cl.: B21C 47/26, C21D 8/02, C21D 9/46, C22C 38/00, C22C 38/02, C22C 38/04, C22C 38/06, C22C 38/08, C22C 38/12, C22C 38/14, C22C 38/18, C22C 38/22, C22C 38/28, C22C 38/32, C22C 38/34, C22C 38/38, C23C 2/02, C23C 2/06, C23C 2/12, B21B 1/02

(54) **HOT PRESS FORMED MEMBER AND METHOD FOR MANUFACTURING THE MEMBER**
HEISSPRESSGEFORMTES ELEMENT SOWIE VERFAHREN ZUR HERSTELLUNG DES ELEMENTS
ÉLÉMENT FORMÉ PAR PRESSAGE À CHAUD ET PROCÉDÉ DE FABRICATION DE L'ÉLÉMENT

(43) Date of publication of application: 21.05.2014
(73) Proprietor: POSCO, Pohang Kyungsangbook-do 790-300 (KR)
(72) Inventor: LEE, Kyoo-Young, Gwangyang-si Jeollanam-do 545-711 (KR); OH, Jin-Keun, Gwangyang-si Jeollanam-do 545-711 (KR); KIM, Jong-Sang, Gwangyang-si Jeollanam-do 545-711 (KR); HAN, Tae-Kyo, Gwangyang-si Jeollanam-do 545-711 (KR)
(74) Representative: Potter Clarkson
(86) International application number: PCT/KR2011/005242
(87) International publication number: WO 2013/012103

(56) References cited:
- EP-A1- 2 325 346
- EP-A1- 2 719 786
- WO-A1-2007/129676
- JP-A- 2007 113 100
- JP-A- 2007 113 100
- KR-A- 20090 101 684
- KR-A- 20100 091 243
- KR-A- 20100 091 243
- US-A- 5 454 887
- US-A1- 2009 238 715

## Description

### [Technical Field]

The present disclosure relates to a hot-press formed member , and a method for manufacturing such a member. The invention is of benefit for manufacturing high-strength and high-ductility products suitable for impact members and crashworthy members of automobiles through a hot press forming process.

### [Background Art]

Recently, safety regulations for protecting automobile occupants and fuel efficiency regulations for protecting the environment have been greatly tightened, and social requirements for vehicle weight reductions have markedly increased. The use of high-strength steel sheets is necessary to reduce the weight of automotive parts while maintaining the rigidity thereof and the crash safety of automobiles.

However, if steel sheets for automobiles are improved in strength, the yield strength thereof is inevitably increased, and the elongation thereof is reduced. These factors significantly lower the formability of such steel sheets. In addition, due to excessive spring-back in high-strength steel sheets, the dimensions of components formed of high-strength steel sheets may be varied after a forming process. That is, the shape fixability of components may be lowered.

To address these limitations, advanced high strength steel (AHSS), such as dual phase (DP) steel in which martensite is included in a ferrite matrix to lower the yield ratio thereof and transformation induced plasticity (TRIP) steel in which bainite and retained austenite are included in a ferrite matrix to markedly increase the strength-elongation balance thereof, have been developed and commercialized.

However, such steel sheets have a tensile strength of about 500 MPa to 1,000 MPa which may be insufficient to satisfy current rigidity and crash safety requirements while allowing for the lightening of automobiles.

Therefore, a steel forming method known as hot press forming has been commercialized to overcome such limitations and realize ultra high-strength automotive components. In the hot press forming method, after blanking, a steel sheet is subjected to heating to an Ac₃ temperature or higher for transformation into austenite, extracting, press forming, and die quenching, so as to form a martensite or mixed martensite-bainite microstructure. Ultra high-strength members having a tensile strength of 1 GPa or greater and high dimensional precision owing to high-temperature forming can be obtained using the hot press forming method.

Although such a hot press forming method of the related art is suitable for satisfying rigidity and crash safety requirements while lightening automotive components, final products have an elongation of 10% or less. That is, final products have a very low level of ductility. In other words, components manufactured by a hot press forming method may be used as impact members in automobiles, but may not be suitable for use as crashworthy members that absorb crash energy to protect vehicle occupants in a crash.

KR20100091243 A discloses a high-strength part and process for producing the same. EP2719786 A1 is a prior art document falling under Art. 54 (3) EPC and discloses a hot press molded article, method for producing same, and thin steel sheet for hot press molding.

Therefore, to use hot-press formed members as crashworthy members of automobiles, research into members having a high degree of ductility after being hot-press formed and steel sheets for forming such members through a hot press forming process is required.

### [Disclosure]

### [Technical Problem]

Aspects of the present invention may provide a hot-press formed member having high strength and high ductility and methods for manufacturing the member.

### [Technical Solution]

According to an example of the present disclosure not specifically claimed herein, a steel sheet for hot press forming may include, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities.

According to another example of the present disclosure also not specifically claimed herein, a method for manufacturing a steel sheet for hot press forming may include: heating a steel slab to a temperature within a range of 1100°C to 1300°C, the steel slab including, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities; performing a finish hot-rolling process at a temperature within a range of an Ar₃ transformation point to 950°C to form a steel sheet; and coiling the steel sheet at a temperature within a range of Mₛ to 720°C.

According to an aspect of the present invention, a hot-press formed member consist of, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities, optionally further consisting of at least one selected from the group consisting of Mo: 0.5% or less, excluding 0%, Cr: 1.5% or less, excluding 0%, Ni: 0.5% or less, excluding 0%, Nb: 0.005% to 0.1%, and V: 0.005% to 0.1% optionally further consisting of a combination of B: 0.005% or less, excluding 0%, and Ti: 0.06% or less, excluding 0%, wherein the hot-press formed member has a dual phase microstructure formed by bainite and retained austenite.

According to another aspect of the present invention, a method for manufacturing a hot-press formed member having a dual phase microstructure formed by bainite and retained austenite, includes: heating a steel sheet to a temperature equal to or higher than Ac₃, the steel sheet consisting of, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities, optionally further consisting of at least one selected from the group consisting of Mo: 0.5% or less, excluding 0%, Cr: 1.5% or less, excluding 0%, Ni: 0.5% or less, excluding 0%, Nb: 0.005% to 0.1%, and V: 0.005% to 0.1%, optionally further consisting of a combination of B: 0.005% or less, excluding 0%, and Ti: 0.06% or less, excluding 0%; hot-press forming the heated steel sheet; cooling the hot-press formed steel sheet to a temperature range of Mₛ to 550°C at a rate of 20°C/sec or higher; and heat-treating the cooled steel sheet at a temperature within a range of Mₛ to 550°C in a heating furnace.

### [Advantageous Effects]

Disclosed herein is a high-strength, high-ductility steel sheet for hot press forming. The present disclosure also provides a member formed using the steel sheet and having a dual phase microstructure constituted by bainite and retained austenite and a TS(MPa)^{∗}El(%) value of 25,000 MPa% or greater. Since the member has high ductility as well as high strength, the member may be usefully used as a crashworthy member of an automobile.

### [Description of Drawings]

FIG. 1 is a temperature-time graph illustrating manufacturing processes of a hot-press formed member according to an embodiment of the present disclosure.
FIGS. 2A to 2C are images showing microstructures of hot-press formed members according to cooling rates after a forming process in a method for manufacturing a hot-press formed member, in which FIG. 2A is the case of a cooling rate of 30°C/sec, FIG. 2B is the case of a cooling rate of 5°C/sec, and FIG. 2C is an enlarged image of FIG. 2B.

### [Best Mode]

Embodiments and examples of the present invention provide a method for manufacturing a formed member having a high degree of ductility as well as high strength for use as a crashworthy member of an automobile. A steel sheet disclosed herein has a high degree of ductility for use in manufacturing such a formed member. In detail, the present disclosure provides four categories: a steel sheet for hot press forming having a high degree of ductility, a method for manufacturing the steel sheet, a hot-press formed member, and a method for manufacturing the hot-press formed member.

### (Steel sheet for hot press forming)

Hereinafter, a steel sheet for hot press forming will be described in detail.

The steel sheet for hot press forming has a high degree of ductility as well as a high degree of strength so that a member formed of the steel sheet through a hot press forming process may have a high degree of ductility and a high degree of strength. The steel sheet for hot press forming includes, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities.

Carbon (C) is an element included in the steel sheet to enhance the strength thereof. Furthermore, in the embodiment of the present disclosure, carbon (C) is diffused into retained austenite by elements such as silicon (Si) to stabilize the retained austenite and thus to prevent transformation to martensite. The steel sheet for hot press forming may include 0.3 wt% to 1.0 wt% of carbon (C). If the carbon content is less than 0.3%, the amount of retained austenite is low after forming, and thus it may be difficult to guarantee both strength and ductility. If the carbon content is greater than 1.0%, bainite transformation is markedly slowed, and the formation of pearlite is facilitated, thereby deteriorating properties of the steel sheet.

Manganese (Mn) is included in the steel sheet to prevent red shortness caused by FeS formed by sulfur (S) inevitably included in the steel sheet during a manufacturing process. The content of manganese (M) may be within the range of 0.01% to 4.0%. If the content of manganese (M) is less than 0.01%, red shortness may be caused by FeS. If the content of manganese (M) is greater than 4.0%, bainite transformation may be slowed to increase the time required for a heat treatment in a hot press forming process. As a result, the productivity of the hot press forming process may be lowered, and the manufacturing cost of the steel sheet may be increased.

Silicon (Si) is an element included in the steel sheet to guarantee the ductility of a final product. Silicon (Si) facilitates ferrite transformation and diffuses carbon (C) into retained austenite to stabilize the retained austenite by an increased amount of carbon (C) in the retained austenite, thereby preventing transformation to martensite. The content of silicon (Si) may be within the range of 1.0 wt% to 2.0 wt%. If the content of silicon (Si) is less than 1.0%, the effect of stabilizing retained austenite may be poor. If the content of silicon (Si) is greater than 2.0%, the rolling characteristics of the steel sheet may be deteriorated. For example, the steel sheet may be cracked during a rolling process. Therefore, the upper limit of the content of silicon (Si) is set as 2.0%.

Aluminum (Al) removes oxygen from the steel sheet to prevent the inclusion of nonmetallic substances therein during solidification. In addition, like silicon (Si), aluminum (Al) facilitates the diffusion of carbon (C) into retained austenite to stabilize the retained austenite. The content of aluminum (Al) may be within the range of 0.01% to 2.0%. If the content of aluminum (Al) is less than 0.01%, oxygen may be insufficiently removed, and thus it may be difficult to prevent the inclusion of nonmetallic substances. If the content of aluminum (Al) is greater than 2.0%, the unit cost of steel making may be increased.

Sulfur (S) is an element inevitably included in the steel sheet during a manufacturing process thereof. Sulfur (S) combines with iron (Fe) to form FeS causing red shortness. Therefore, it may be necessary to keep the content of sulfur (S) as low as possible. For example, the content of sulfur (S) may be limited to 0.015% or less. Nitrogen (N) is an element inevitably included in the steel sheet during a manufacturing process. The content of nitrogen (N) may be kept as low as possible. For example, the content of nitrogen (N) may be limited to 0.01% or less.

In addition to the above-mentioned elements, the steel sheet for hot press forming may further include at least one element selected from the group consisting of Mo: 0.5% or less (excluding 0%), Cr: 1.5% or less (excluding 0%), Ni: 0.5% or less (excluding 0%), Nb: 0.005% to 0.1%, and V: 0.005% to 0.1%.

Molybdenum (Mo) may be added to the steel sheet to suppress the formation of pearlite. Since molybdenum (Mo) is relatively expensive and may increase the manufacturing cost of the steel sheet, 0.5 wt% or less of molybdenum (Mo) may be added.

Chromium (Cr) may be added to the steel sheet to suppress the formation of ferrite and expand bainite transformation. If the content of chromium (Cr) is greater than 1.5 wt%, chromium carbide may be formed to lower the amount of dissolved carbon (C). Therefore, 1.5 wt% or less of chromium (Cr) may be added.

Nickel (Ni) may be added to increase the faction of austenite and the hardenability of the steel sheet. Since nickel (Ni) is expensive and increases the manufacturing cost of the steel sheet, 0.5 wt% or less of nickel (Ni) may be added.

Niobium (Nb) may be added to improve the strength, grain refining characteristics, and ductility of the steel sheet. During reheating, niobium (Nb) suppresses grain growth, and during cooling, niobium (Nb) delays transformation of austenite into ferrite. 0.005 wt% to 0.1 wt% of niobium (Nb) may be added. If the content of niobium (Nb) is less than 0.005%, it is difficult to assure the effect of grain refinement, and if the content of niobium (Nb) is greater than 0.1%, carbonitrides may excessively precipitate to cause delayed fractures in the steel sheet or decrease the workability of the steel sheet.

Vanadium (V) may be added to improve the strength, grain refining characteristics, and hardenability of the steel sheet. 0.005 wt% to 0.1 wt% of vanadium (V) may be added. If the content of vanadium (V) is less than 0.005%, such effects may not be obtained, and if the content of vanadium (V) is greater than 0.1%, carbonitrides may excessively precipitate to cause delayed fractures in the steel sheet or decrease the workability of the steel sheet.

In addition, the steel sheet for hot press forming may further include B: 0.005% or less (excluding 0%) and Ti: 0.06% or less (excluding 0%).

Boron (B) may be added to suppress the formation of ferrite. If the content of boron (B) is greater than 0.005 wt%, boron (B) may combine with iron (Fe) or carbon (C) to form a compound facilitating the formation of ferrite. Therefore, 0.005 wt% of less of boron (B) may be added.

Titanium (Ti) may be added to maximize the effect of boron (B). Titanium (Ti) combines with nitrogen (N) existing as an impurity in the steel sheet to form TiN, and thus boron (B) may not combine with nitrogen (N). Therefore, the formation of ferrite may be suppressed by boron (B). This effect may be assured by adding 0.06 wt% or less of titanium (Ti).

The steel sheet may be a hot-rolled or cold-rolled steel sheet. For example, the steel sheet may be a cold-rolled steel sheet coated with a plating layer for improving corrosion resistance and suppressing the formation of a surface oxide layer.

Since the steel sheet for hot press forming has high strength and high ductility owing to the above-described composition, the steel sheet may be usefully used to manufacture hot-press formed members (described later) having high strength and ductility.

### (Method for manufacturing steel sheet for hot press forming)

Hereafter, a method for manufacturing a steel sheet for hot press forming will be described in detail. This is an exemplary example for manufacturing a steel sheet suitable for manufacturing a hot-press formed member having improved ductility.

The method for manufacturing a steel sheet for hot press forming includes: heating a steel slab to a temperature within a range of 1100°C to 1300°C, the steel slab including, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities; performing a finish hot-rolling process at a temperature within a range of Ar₃ transformation point to 950°C to form a steel sheet; and coiling the steel sheet at a temperature within a range of Mₛ to 720°C.

If the steel slab is heated to a temperature lower than 1100°C, the continuous-casting structure of the steel slab may be insufficiently uniformized, and it may be difficult to assure a finish rolling temperature. If the steel slab is heated to a temperature greater than 1300°C, the size of crystal grains and the possibility of surface oxidation may increase to deteriorate the strength and surface properties of the steel slab. Therefore, the steel slab may be heated to a temperature within a range of 1100°C to 1300°C. If the finish hot-rolling temperature is lower than Ar₃ transformation point, dual phase rolling may occur to result in hot-rolling mixed grain sizes, and if the finish hot-rolling temperature is higher than 950°C, crystal grains may be coarsened and surface oxidation may occur during the finish hot-rolling process. Therefore, the finish hot-rolling temperature may be within the range of the Ar₃ transformation point to 950°C. In addition, if the coiling temperature is lower than Mₛ, austenite may transform to martensite to decrease the ductility of the steel sheet and thus to make it difficult to perform a hot coiling process on the steel sheet. If the coiling temperature is higher than 720°C, a thick surface oxide layer may be formed on the steel sheet together with internal oxidation in the steel sheet. Therefore, the coiling temperature may be within the range of Mₛ to 720°C.

The method for manufacturing a steel sheet for hot press forming may include: heating a steel slab to a temperature within a range of 1100°C to 1300°C, the steel slab including, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities; performing a finish hot-rolling process at a temperature within a range of Ar₃ transformation point to 950°C to form a steel sheet; coiling the steel sheet at a temperature within a range of Mₛ to 720°C; pickling the steel sheet; cold-rolling the steel sheet; continuously annealing the steel sheet at a temperature within a range of 750°C to 900°C; and overaging the steel sheet at a temperature within a range of Mₛ to 550°C.

The pickling of the steel sheet is performed to remove surface oxides formed during the heating and finish hot-rolling processes. Thereafter, the cold-rolling process is performed. If the continuous annealing temperature for the cold-rolled steel sheet is lower than 750°C, recrystallization may occur insufficiently, and thus a desired degree of workability of the steel sheet may not be obtained. If the continuous annealing temperature is higher than 900°C, it may difficult to heat the steel sheet to the continuous annealing temperature due to the limitation of heating equipment. In addition, if the overaging temperature is lower than Mₛ, martensite may be formed to excessively increase the strength of the steel sheet and negatively affect the ductility of the steel sheet. Therefore, before a hot press forming process, blanking may not be easily performed. If the overaging temperature is higher than 550°C, the processability of the steel sheet may be lowered due to roll surface deterioration in an annealing furnace, and intended carbide precipitation and bainite transformation may not occur in the overaging process.

The method for manufacturing a steel sheet for hot press forming may include: heating a steel slab to a temperature range of 1100°C to 1300°C, the steel slab including, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities; performing a finish hot-rolling process at a temperature within a range of Ar₃ transformation point to 950°C to form a steel sheet; coiling the steel sheet at a temperature within a range of Mₛ to 720°C; pickling the steel sheet; cold-rolling the steel sheet; continuously annealing the steel sheet at a temperature within a range of 750°C to 900°C; overaging the steel sheet at a temperature within a range of Mₛ to 550°C; and plating the overaged steel sheet by any one of hot-dip galvanizing, galvannealing, electro galvanizing, and hot-dip aluminizing.

A hot-dip galvanized steel sheet may be manufactured by dipping a cold-rolling steel sheet in a galvanizing bath. A galvannealed steel sheet may be manufactured by dipping a cold-rolled steel sheet in a plating bath and performing an alloying heat-treatment process on the steel sheet. An electro-galvanized steel sheet may be manufactured by performing an electro galvanizing process or a Zn-Fe electroplating process on a cold-rolled steel sheet in a continuous electroplating line. A hot-dip aluminized steel sheet may be manufactured by heating a cold-rolled steel sheet, dipping the steel sheet in an aluminum plating bath, and cooling the steel sheet at room temperature at a cooling rate of 5°C/sec to 15°C/sec.

The steel slab may further include at least one selected from the group consisting of Mo: 0.5% or less (excluding 0%), Cr: 1.5% or less (excluding 0%), Ni: 0.5% or less (excluding 0%), Nb: 0.005% to 0.1%, and V: 0.005% to 0.1%. In addition, the steel slab may further include B: 0.005% or less (excluding 0%) and Ti: 0.06% or less (excluding 0%).

### (Hot-press formed member)

Hereinafter, a hot-press formed member will be described in detail according to an embodiment of the present invention.

The hot-press formed member has high ductility and high strength. For this, the hot-press formed member includes, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities. The hot-press formed member may have a microstructure formed of bainite and retained austenite without martensite.

The hot-press formed member may further include at least one selected from the group consisting of Mo: 0.5% or less (excluding 0%), Cr: 1.5% or less (excluding 0%), Ni: 0.5% or less (excluding 0%), Nb: 0.005% to 0.1%, and V: 0.005% to 0.1%. In addition, the hot-press formed member may further include B: 0.005% or less (excluding 0%) and Ti: 0.06% or less (excluding 0%).

Hot-press formed members of the related art are manufactured to have ultra high strength, and thus martensite is requisitely formed therein. However, martensite lowers the ductility of such hot-press formed members and thus makes such hot-press formed members unsuitable to be used as crashworthy members of automobiles. Therefore, in the embodiment of the present disclosure, the formation of martensite in the hot-press formed member is suppressed, and the amount of retained austenite is increased. Thus, the hot-press formed member has dual phases: bainite and retained austenite.

The hot-press formed member having the above-mentioned composition and microstructure has good strength-ductility balance. For example, TS^{∗}El of the hot-press formed member may be 25,000 or greater so as to be used as a crashworthy member of an automobile as well as being used as an impact member, where TS denotes tensile strength [MPa] and El denotes elongation [%].

### (Method for manufacturing hot-press formed member)

Hereinafter, a method for manufacturing a hot-press formed member will be described in detail according to an embodiment of the present invention.

The method is for performing a hot press forming process on the above-described steel sheet to provide an ultra high-strength automotive component having high ductility. For this, the method includes: heating a steel sheet to a temperature equal to or higher than Ac₃, the steel sheet including, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities; hot-press forming the heated steel sheet; cooling the hot-press formed steel sheet to a temperature range of Mₛ to 550°C at a rate of 20°C/sec or higher; and heat-treating the cooled steel sheet in a heating furnace heated at a temperature within a range of Mₛ to 550°C.

The steel sheet may further include at least one selected from the group consisting of Mo: 0.5% or less (excluding 0%), Cr: 1.5% or less (excluding 0%), Ni: 0.5% or less (excluding 0%), Nb: 0.005% to 0.1%, and V: 0.005% to 0.1%. In addition, the steel sheet may further include B: 0.005% or less (excluding 0%) and Ti: 0.06% or less (excluding 0%). The steel sheet may be one of a hot-rolled steel sheet, a cold-rolled steel sheet, and a plated cold-rolled steel sheet coated with a plating layer.

In the method for manufacturing a hot-press formed member according to the embodiment of the present invention, the heat-treating after the hot-press forming is controlled differently as compared with the case of the related art, so as to manufacture a hot-press formed member having a different microstructure for improving ductility as compared with a hot-press formed member of the related art. That is, in the related art, heat-treatment conditions are adjusted to form martensite as a main microstructure to finally obtain an ultra high-strength member. However, since such a technique of the related art is not suitable to manufacture a highly ductile member usable as a crashworthy member of an automobile, the inventors have suggested heat treatment conditions for forming a microstructure constituted by bainite and retained austenite without martensite.

First, the steel sheet is heated to a temperature equal to Ac₃ or higher for transformation to austenite, and is then hot-press formed.

The heat-treatment conditions after the hot-press forming have a major effect on determining the microstructure of a product. In the related art, generally, a hot-press formed steel sheet is directly die-quenched to a temperature equal to or lower than Mₛ so as to form martensite as a main microstructure in a final product and thus to enhance the strength of the final product.

However, in the embodiment of the present invention, martensite is excluded from the microstructure of a final product so as to improve the ductility of the final product while maintaining the strength of the final product at a level suitable for weight reduction. To this end, instead of cooling the hot-press formed steel sheet directly to room temperature equal to or lower than Mₛ, the hot-press formed steel sheet is cooled to a temperature range of Mₛ to 550°C, and heat-treated in a heating furnace at a temperature within a range of Mₛ to 550°C so as to cause the hot-press formed steel sheet to undergo transformation to bainite. If the steel sheet is cooled to a temperature equal to or lower than Mₛ, martensite may be formed to lower the ductility of the steel sheet, and if the steel sheet is cooled to a temperature higher than 550°C, pearlite may be formed to deteriorate properties of the steel sheet. Therefore, the cooling rate is adjusted to be within the range of Mₛ to 550°C to form a dual phase microstructure constituted by bainite and retained austenite.

In the bainite formed as described above, Fe₃C carbide may not be formed because elements such as silicon (Si) are sufficiently included in the steel sheet to diffuse carbon (C) into the retained austenite. That is, carbon (C) does not form carbides but is dissolved in the retained austenite to stabilize the retained austenite and thus to lower Mₛ. Therefore, in the next cooling process, transformation to martensite is suppressed. Therefore, in a final product, the retained austenite remains instead of undergoing transformation to martensite, thereby improving ductility.

The cooling rate may be 20°C/sec or higher. If the cooling rate is lower than 20°C/sec, transformation to pearlite may easily occur to lower properties of a final product. Referring to FIG. 2A, bainite was formed at a cooling rate of 30°C/sec. However, referring to FIGS. 2B and 2C, a pearlite structure in which ferrite and Fe₃C were layered was formed at a cooling rate of 5°C/sec.

For example, the above-described processes for manufacturing a hot-press formed member according to the embodiment of the present disclosure may be summarized as follows. First, a steel sheet is inserted in a heating furnace to heat the steel sheet to Ac₃ or higher for forming austenite, and then the heated steel sheet is hot-press formed. After the hot press forming, the steel sheet is cooled to a temperature range of Mₛ to 550°C at a cooling rate of 20°C/sec or higher so as not to form pearlite, and is then heat-treated in a heating furnace at a temperature within a range of Mₛ to 550°C. These processes are for transformation to bainite, and during the processes, carbon (C) diffuses into austenite to lower Mₛ. Although a hot-press formed member manufactured through the above-described processes is cooled to room temperature without any controlling, transformation to martensite does not occur. That is, a dual phase microstructure constituted by bainite and retained austenite may be obtained.

Hereinafter, the embodiments of the present invention will be described more specifically according to examples. The following examples are merely provided to allow for a clear understanding of the present disclosure, rather than to limit the scope thereof.

### [Mode for Invention]

### (Examples)

Steel ingots 90 mm in length and 175 mm in width having compositions shown in Table 1 were manufactured by vacuum melting, and were then re-heated at 1200°C for 1 hour. Thereafter, the steel ingots were hot-rolled to obtain steel sheets having a thickness of 3 mm. At that time, a finish hot-rolling temperature was Ar₃ or higher. Then, after cooling the steel sheets, the steel sheets were inserted into a heating furnace previously heated to 600°C and left in the heating furnace for 1 hour. Thereafter, the steel sheets were cooled in the heating furnace to simulate hot coiling. Next, the steel sheets were cold-rolled at a reduction ratio of 60% to a thickness of 1.2 mm and were annealed at 900°C. Then, the steel sheets were allowed to undergo bainite transformation at 400°C. In Table 1, the contents of elements are given in wt% except for the contents of sulfur (S) and nitrogen (N) given in ppm.

**[Table 1]**

| Steels | C | Si | Mn | Al | Mo | Cr | Ni | Ti | B | Nb | V | S | N |
|---|---|---|---|---|---|---|---|---|---|---|---|---|---|
| IS* 1 | 0.40 | 1.51 | 3.01 | 0.04 | | | | | | | | 30 | 20 |
| IS 2 | 0.63 | 1.49 | 0.72 | 0.50 | | | | | | | | 20 | 20 |
| IS 3 | 0.61 | 1.52 | 0.63 | 0.51 | | | 0.30 | | | | | 30 | 20 |
| IS 4 | 0.61 | 1.50 | 0.65 | 0.50 | | | | | | 0.015 | | 30 | 20 |
| IS 5 | 0.62 | 1.49 | 1.61 | 1.53 | | | | | | | 0.02 | 30 | 20 |
| IS 6 | 0.60 | 1.50 | 2.91 | 0.04 | 0.25 | 1.20 | | | | | | 20 | 20 |
| IS 7 | 0.71 | 1.47 | 0.7 | 0.52 | | | | 0.010 | 0.002 | | | 20 | 20 |
| IS 8 | 0.68 | 1.48 | 0.71 | 0.04 | 0.24 | | | | | | | 30 | 20 |
| IS 9 | 0.70 | 1.15 | 0.72 | 0.51 | 0.24 | | | | | | | 30 | 20 |
| IS 10 | 0.71 | 1.15 | 0.71 | 0.04 | 0.24 | | | 0.010 | 0.002 | | | 30 | 20 |
| IS 11 | 0.69 | 1.55 | 0.18 | 0.04 | 0.24 | 0.50 | | 0.010 | 0.002 | | | 30 | 20 |
| IS 12 | 0.82 | 1.49 | 0.51 | 0.54 | | | | | | | | 30 | 20 |
| IS 13 | 0.82 | 1.51 | 1.01 | 0.53 | | | | | | | | 30 | 20 |
| CS** 1 | 0.23 | 1.5 | 1.5 | 0.04 | | | | | | | | 30 | 20 |
| CS 2 | 0.20 | 0.5 | 1.5 | 0.03 | | | | | | | | 30 | 20 |
| CS 3 | 0.22 | 1.5 | 2 | 0.03 | 0.20 | | | | | | | 20 | 20 |
| CS 4 | 0.68 | 0.42 | 0.70 | 0.52 | | | | | | | | 20 | 20 |

| | | | | | | | | | | | | | |
|---|---|---|---|---|---|---|---|---|---|---|---|---|---|
| *IS: Inventive Steel, **CS: Comparative Steel | | | | | | | | | | | | | |

To simulate a heat treatment in a heating furnace during a hot press forming process, the 1.2 mm thickness steel sheets manufactured as described above were heated to a temperature of 900°C and maintained at the temperature for 30 seconds. Then, the steel sheets were cooled to cooling temperatures at a rate of 30°C/sec. Next, the steel sheets were inserted into a heating furnace and heat-treated in the heating furnace at the same temperatures as the cooling temperatures for 400 seconds to 10,800 seconds. Thereafter, the steel sheets were air-cooled. In this way, hot-press formed members were obtained. The process conditions and mechanical properties of the hot-press formed members are shown in Table 2 below.

**[Table 2]**

| Steels | Cooling Rate (°C/sec) | Cooling Temperature (°C) | Time (sec) | YS (MPa) | TS (MPa) | El (%) | TS^{∗}El (MPa%) | Mₛ (°C) |
|---|---|---|---|---|---|---|---|---|
| Is* 1 | 30 | 400 | 3600 | 732 | 1265 | 28 | 35420 | 295 |
| IS 2 | 30 | 400 | 3600 | 899 | 1187 | 39 | 46244 | 298 |
| IS 3 | 30 | 400 | 3600 | 869 | 1196 | 37 | 44252 | 302 |
| IS 4 | 30 | 400 | 3600 | 915 | 1289 | 35 | 45115 | 307 |
| IS 5 | 30 | 400 | 3600 | 883 | 1185 | 36 | 42660 | 272 |
| IS 6 | 30 | 400 | 10800 | 856 | 1420 | 26 | 36920 | 199 |
| | 30 | 300 | 10800 | 985 | 1610 | 22 | 35420 | 199 |
| IS 7 | 30 | 400 | 3600 | 900 | 1185 | 40 | 46923 | 273 |
| | 5 | 400 | 3600 | 719 | 1128 | 11 | 12408 | 273 |
| IS 8 | 30 | 400 | 600 | 816 | 1310 | 21 | 27510 | 280 |
| IS 9 | 30 | 400 | 600 | 915 | 1240 | 29 | 35960 | 277 |
| IS 10 | 30 | 400 | 600 | 845 | 1318 | 25 | 32950 | 270 |
| IS 11 | 30 | 400 | 600 | 940 | 1288 | 26 | 33488 | 280 |
| IS 12 | 30 | 400 | 3600 | 881 | 1229 | 35 | 43556 | 245 |
| IS 13 | 30 | 400 | 3600 | 725 | 1306 | 39 | 50934 | 228 |
| CS** 1 | 30 | 400 | 3600 | 640 | 1125 | 15 | 16875 | 399 |
| | 30 | 250 | 3600 | 1295 | 1511 | 6 | 9066 | 399 |
| CS 2 | 30 | 250 | 3600 | 1220 | 1450 | 7 | 10150 | 420 |
| CS 3 | 30 | 250 | 3600 | 1280 | 1490 | 6 | 8940 | 384 |
| CS 4 | 30 | 400 | 3600 | 870 | 1201 | 16 | 19216 | 295 |

| | | | | | | | | |
|---|---|---|---|---|---|---|---|---|
| *IS: Inventive Steel, **CS: Comparative Steel | | | | | | | | |

Since TS^{∗}El of Comparative Steel 1 cooled at a cooling rate of 400°C is 16,785 MPa%, Comparative Steel 1 is not suitable as a crashworthy member of an automobile. The reason for this may be that the insufficient content of carbon (C) led to failure in stabilizing retained austenite. In the case that the cooling rate was 250°C, Comparative Steel 1 was cooled to a temperature lower than Mₛ to result in a large amount of transformation to martensite, and thus Comparative Steel 1 had high strength but low ductility. In this case, TS^{∗}El of Comparative Steel 1 is 9,066 MPa%, and Comparative Steel 1 is not suitable to form a crashworthy member of an automobile.

The carbon (C) content and silicon (Si) content of Comparative Steel 2 are also not sufficient to stabilize retained austenite, and the cooling temperature of Comparative Steel 2 is equal to or lower than Mₛ to result in transformation to martensite. Therefore, Comparative Steel 2 has low ductility, and TS^{∗}El thereof is low at 10,150 MPa%. Comparative Steel 3 also has an insufficient content of carbon (C), and the cooling temperature of Comparative Steel 3 is equal to or lower than Mₛ. Therefore, TS^{∗}El of Comparative Steel 3 is low at 8,940 MPa%, and Comparative Steel 3 is not suitable to form a crashworthy member of an automobile.

Although Comparative Steel 4 has a sufficient content of carbon (C), the silicon (Si) content of Comparative Steel 4 is not sufficient to fully diffuse carbon (C) into retained austenite. Therefore, although TS^{∗}El of Comparative Steel 4 is relatively high at 19,216 MPa% as compared with other comparative steels, TS^{∗}El of Comparative Steel 4 is not greater than 25,000 MPa%. That is, Comparative Steel 4 is not suitable for forming a crashworthy member of an automobile.

Samples of Inventive Steel 7 having a composition within the range of the present disclosure were cooled at a cooling rate of 30°C/sec and at a cooling rate of 5°C/sec, respectively. In the case that the cooling rate was 30°C/sec, TS^{∗}El of Inventive Steel 7 was high at 46,923 MPa% and suitable for a crashworthy member of an automobile. However, in the case that the cooling rate was 5°C/sec, TS^{∗}El of Inventive Steel 7 was low at 12, 480 MPa% and not suitable for a crashworthy member of an automobile. The reason for this may be that the low cooling rate led to the formation of pearlite as shown in FIGS. 2A to 2C and deterioration of properties thereof.

## Claims

1. A hot-press formed member consisting of, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities, optionally further consisting of at least one selected from the group consisting of Mo: 0.5% or less, excluding 0%, Cr: 1.5 or less, excluding 0%, Ni: 0.5 or less, excluding 0%, Nb: 0.005% to 0.1%, and V: 0.005% to 0.1%, optionally further consisting of a combination of B: 0.005% or less, excluding 0%, and Ti: 0.06% or less, excluding 0%, wherein the hot-press formed member has a dual phase microstructure formed by bainite and retained austenite.

2. The hot-press formed member of claim 1, wherein the hot-press formed member has a TS(MPa)^{∗}El(%) value of 25,000 MPa% or greater, where TS denotes tensile strength in MPa and El denotes elongation in %.

3. A method for manufacturing a hot-press formed member having a dual phase microstructure formed by bainite and retained austenite, the method comprising:
heating a steel sheet to a temperature equal to or higher than Ac₃, the steel sheet consisting of, by wt%, C: 0.3% to 1.0%, Mn: 0.01% to 4.0%, Si: 1.0% to 2.0%, Al: 0.01% to 2.0%, S: 0.015% or less, N: 0.01% or less, and the balance of Fe and inevitable impurities, optionally further consisting of at least one selected from the group consisting of Mo: 0.5% or less, excluding 0%, Cr: 1.5% or less, excluding 0%, Ni: 0.5% or less, excluding 0%, Nb: 0.005% to 0.1%, and V: 0.005% to 0.1%, optionally further consisting of a combination of B: 0.005% or less, excluding 0%, and Ti: 0.06% or less, excluding 0%;
hot-press forming the heated steel sheet;
cooling the hot-press formed steel sheet to a temperature range of Mₛ to 550°C at a rate of 20°C/sec or higher; and
heat-treating the cooled steel sheet at a temperature within a range of Mₛ to 550°C in a heating furnace.

4. The method of claim 3, wherein the steel sheet is one of a hot-rolled steel sheet, a cold-rolled steel sheet, and a plated cold-rolled steel sheet coated with a plating layer.

## Patentansprüche

1. Heißpressformteil, das in Gew.-% aus Folgendem besteht: C: 0,3 % bis 1,0 %, Mn: 0,01 % bis 4,0 %, Si: 1,0 bis 2 %, Al: 0,01 % bis 2,0 %, S: 0,015 % oder weniger, N: 0,01 % oder weniger, und wobei der Rest aus Fe und unvermeidlichen Verunreinigungen besteht, gegebenenfalls ferner bestehend aus mindestens einem aus der Gruppe bestehend aus Mo: 0,5 % oder weniger, ausgenommen 0 %, Cr: 1,5 % oder weniger, ausgenommen 0 %, Ni: 0,5 % oder weniger, ausgenommen 0 %, Nb: 0,005 % bis 0,1 % und V: 0,005 % bis 0,1 %, gegebenenfalls ferner bestehend aus einer Kombination von B: 0,005 % oder weniger, ausgenommen 0 %, und Ti: 0,06 % oder weniger, ausgenommen 0 %, wobei das Heißpressformteil eine aus Bainit und Restaustenit gebildete Zweiphasenmikrostruktur aufweist.

2. Heißpressformteil nach Anspruch 1, wobei das Heißpressformteil einen TS(MPa)^{∗}E1(%)-Wert von 25.000 MPa.-% oder mehr aufweist, wobei TS die Zugfestigkeit in MPa bezeichnet und E1 die Dehnung in % bezeichnet.

3. Verfahren zur Herstellung eines Heißpressformteils mit einer aus Bainit und Restaustenit gebildeten Zweiphasenmikrostruktur, wobei das Verfahren Folgendes umfasst:
Erwärmen eines Stahlblechs auf eine Temperatur, die gleich oder höher als AC₃ ist, wobei das Stahlblech in Gew.-% aus Folgendem besteht C: 0,3 % bis 1,0 %, Mn: 0,01 % bis 4,0 %, Si: 1,0 % bis 2,0 %, Al: 0,01 % bis 2,0 %, S: 0,015 % oder weniger, N: 0,01 % oder weniger, und wobei der Rest aus Fe und unvermeidlichen Verunreinigungen besteht, gegebenenfalls ferner bestehend aus mindestens einem aus der Gruppe bestehend aus Mo: 0,5 % oder weniger, ausgenommen 0 %, Cr: 1,50 % oder weniger, ausgenommen 0 %, Ni: 0,5 % oder weniger, ausgenommen 0 %, Nb: 0,005 % bis 0,1 % und V: 0,005 % bis 0,1 %, gegebenenfalls ferner bestehend aus einer Kombination von B: 0,005 % oder weniger, ausgenommen 0 %, und Ti: 0,06 % oder weniger, ausgenommen 0 %;
Heißpressformen des erwärmten Stahlblechs;
Abkühlen des heißpressgeformten Stahlblechs auf einen Temperaturbereich von Mₛ bis 550 °C mit einer Geschwindigkeit von 20 °C/Sek. oder höher; und
Wärmebehandeln des abgekühlten Stahlblechs bei einer Temperatur innerhalb eines Bereichs von Mₛ bis 550 °C in einem Heizofen.

4. Verfahren nach Anspruch 3, wobei das Stahlblech eines von Folgendem ist: ein warmgewalztes Stahlblech, ein kaltgewalztes Stahlblech und ein plattiertes kaltgewalztes Stahlblech, das mit einer Plattierungsschicht beschichtet ist.

## Revendications

1. Élément formé par pressage à chaud constitué, en % en poids, par le C : 0,3 % à 1,0 %, le Mn : 0,01 % à 4,0 %, le Si : 1,0 % à 2,0 %, l'Al : 0,01 % à 2,0 %, le S : 0,015 % ou moins, le N : 0,01 % ou moins et le reste étant du Fe et des impuretés inévitables, étant constitué éventuellement en outre par au moins un élément choisi dans le groupe constitué par le Mo : 0,5 % ou moins, à l'exclusion de 0 %, le Cr : 1,5 ou moins, à l'exclusion de 0 %, le Ni : 0,5 ou moins, à l'exclusion de 0 %, le Nb : 0,005 % à 0,1 % et le V : 0,005 % à 0,1 %, étant constitué éventuellement en outre par une combinaison de B : 0,005 % ou moins, à l'exclusion de 0 % et de Ti : 0,06 % ou moins, à l'exclusion de 0 %, l'élément formé par pressage à chaud comportant une microstructure à deux phases formée par de la bainite et de l'austénite résiduelle.

2. Élément formé par pressage à chaud selon la revendication 1, dans lequel l'élément formé par pressage à chaud comporte une valeur TS(MPa)^{∗}E1(%) égale ou supérieure à 25 000 MPa%, où TS représente la résistance à la traction en MPa et E1 l'allongement en %.

3. Procédé de fabrication d'un élément formé par pressage à chaud comportant une microstructure à deux phases formée par de la bainite et de l'austénite résiduelle, le procédé comprenant :
le chauffage d'une tôle d'acier à une température égale ou supérieure à Ac₃, la tôle d'acier étant constituée, en % en poids, par le C : 0,3 % à 1,0 %, le Mn : 0,01 % à 4,0 %, le Si : 1,0 % à 2,0 %, l'Al : 0,01 % à 2,0 %, le S : 0,015 % ou moins, le N : 0,01 % ou moins, et le reste étant du Fe et des impuretés inévitables, étant constitué éventuellement en outre par au moins un élément choisi dans le groupe constitué par le Mo : 0,5 % ou moins, à l'exclusion de 0 %, le Cr : 1,5 % ou moins, à l'exclusion de 0 %, le Ni : 0,5 % ou moins, à l'exclusion de 0 %, le Nb : 0,005 % à 0,1 % et le V : 0,005 % à 0,1 %, étant constitué éventuellement en outre par une combinaison de B : 0,005 % ou moins, à l'exclusion de 0 %, et de Ti : 0,06 % ou moins, à l'exclusion de 0 % ;
la formation de la tôle d'acier chauffée par pressage à chaud ;
le refroidissement de la tôle d'acier formée par pressage à chaud à une plage de température de Mₛ à 550° C au taux de 20 °C/sec ou plus ; et
le traitement thermiquement de la tôle d'acier refroidie à une température située dans une plage de Mₛ à 550 °C dans un four de chauffage.

4. Procédé selon la revendication 3, dans lequel la tôle d'acier est l'une d'une tôle d'acier laminée à chaud, d'une tôle d'acier laminée à froid et d'une tôle d'acier laminée à froid plaquée revêtue d'une couche de placage.
